

# UNITED STATES PATENT OFFICE.

LOUIS BARTHÉLEMY, OF PARIS, FRANCE.

## EXPLOSIVE.

No. 829,362.

Specification of Letters Patent.

Patented Aug. 21, 1906.

Application filed March 16, 1905. Serial No. 250,368.

*To all whom it may concern:*

Be it known that I, LOUIS BARTHÉLEMY, a citizen of the Republic of France, residing at Paris, France, and whose post-office address 5 is Rue de Provence, No. 62, Paris, France, have invented certain new and useful Improvements in Explosives, of which the following is a full and complete specification, such as will enable those skilled in the art to 10 which it appertains to make and use the same.

The restrictions imposed by marine forwarding agencies or insurance companies make it almost impossible to send explosives 15 to countries beyond the sea. On the other hand, certain explosives can not be easily preserved. Those having a nitroglycerin base exude, and in this case are unquestionably dangerous. Those with a base of chlorate of potash and of vegetable oils harden in 20 a short time under the oxidizing action of the chlorate and soon become useless.

This invention relates to the manufacture 25 of powerful explosives on the spot where they are to be used, and it offers the following advantages: First, it enables the goods to be conveyed under economical conditions by reason of the avoidance of all danger; second, does away with the necessity of keeping 30 quantities in stock, and, third, in case such stocks are rendered necessary insures the perfect preservation of the goods.

The new invention consists in the preparation 35 of harmless mixtures or compositions heretofore unknown which can be conveyed from place to place without danger, and at the moment when they are about to be used they can be mixed with a combustive agent convenient for forming an explosive. I do 40 not say that the method of mixing such harmless compositions with a combustive agent forms part of my invention, for I am well aware that it is a known practice to form explosives by mixing combustible bodies together with oxidizing agents and only at the 45 moment of using the compound for blasting, &c. My invention essentially resides in the preparation of a new and harmless combustible mixture into which on the spot of employment an oxidant is to be incorporated. The oxidizing agent may be some form of nitrate, so as to form a safety explosive, or a 50 chlorate or perchlorate.

The composition of the combustible mix- 55 ture must naturally vary according to the nature of the explosive to be made. It is,

however, composed substantially of a nitrated or non-nitrated hydrocarbon liquid with which the desired proportion of solid nitrated or non-nitrated hydrocarbons is incorporated. The most suitable nitrated hydrocarbon liquids for the preparation of the mixture are orthonitrotoluol and trinitrotoluol. This preparation is made on the base of the principle that paraffin dissolves easily 60 in orthonitrotoluol when liquefied at 60° to 65° centigrade and that it is then easy to incorporate trinitrotoluol.

In case the mixture is to be employed in the preparation of chlorated explosives paraffin is preferable to vegetable oils and other compounds containing a large quantity of carbon, as it remains unaffected in presence of oxidizing agents, which is the reason why chlorated explosives manufactured in this 70 way can be preserved for any length of time. To the combustible paste a certain quantity of metal filings (aluminium, iron, or the like) may be added if it be desired to increase the density of the explosive or the temperature 75 at which detonation takes place. In this manner very stable and entirely harmless pasty mixtures may be made which are quite unaffected by external agents (heat, damp, or the like) and which can be conveyed from place to place with the greatest convenience and safety.

As already stated, the ingredients forming the new product in its preferred composition are paraffin, orthonitrotoluol, and trinitrotoluol, with or without an addition of filings of iron or other metals. The proportions vary according to the strength desired to be obtained by the explosives. By way of an example the following composition may be 85 cited:

|                  | Moderately active. | Strong explosive. |     |
|------------------|--------------------|-------------------|-----|
| Paraffin         | 85                 | 88                | 100 |
| Orthonitrotoluol | 50                 | 18                |     |
| Trinitrotoluol   | 15                 | 18                |     |

To these compositions fifty-one parts of metal filings may be added.

The proportions of the nitrated hydrocarbons can be varied at will between the above-indicated limits according to the desire to make the resulting explosive more or less breaking. The proportions of the paraffin 110 and the metal filings remain preferably unchanged.

- For manufacturing the explosive on the spot where it is to be used all that is necessary is to liquefy the combustible mixture by heating it to about 65° centigrade and mix it with the oxidizing agent bought on the spot or brought separately. It is suitable for a good result to mix about seventy parts of chlorate of potash with thirty parts of the heated and liquefied nitro compound.
- 10 The work is carried out in the simplest manner. If it be desired to manufacture the explosive on a large scale, a pug-mill with a grinder, of wood, and double bottom heated by steam is employed. If it be desired to manufacture only sufficient for daily use, a simple iron pot may be used, which is placed over a water-bath, the two constituents of the explosive being mixed with a wooden stirrer. In this way as much as five kilo-  
20 grams of explosive can be easily made at one

time, the operation only lasting a few minutes.

Having thus described my invention, what I claim is—

1. An explosive consisting of paraffin, orthonitrotoluol and trinitrotoluol.
2. An explosive consisting of paraffin, orthonitrotoluol and trinitrotoluol in substantially the proportions specified.
3. The herein-described process of preparing a compound as the harmless part of a high explosive, which consists in dissolving paraffin in orthonitrotoluol, and then incorporating therewith trinitrotoluol.

In witness whereof I have hereunto set my hand in the presence of two witnesses.

LOUIS BARTHÉLEMY.

Witnesses:

ERIK SOPHIE HICKOK, Jr.,  
ROBERT A. BAKER.